

# United States Patent [19]

Dawson et al.

[11] 3,804,589

[45] Apr. 16, 1974

[54] INCREASING DYE FASTNESS OF SOLVENT DYED SOLVENT SCOUR ED DRIED FABRIC BY STEAMING

[75] Inventors: Ross R. Dawson; William H. Leyking, both of Buffalo, N.Y.

[73] Assignee: The Dow Chemical Company, Midland, Mich.

[22] Filed: Nov. 18, 1969

[21] Appl. No.: 877,828

[52] U.S. Cl. .... 8/165, 8/94, 8/149.1, 8/149.3, 8/17

[51] Int. Cl. .... D06p 5/02

[58] Field of Search..... 8/94, 174, 175

[56] References Cited

UNITED STATES PATENTS

|           |         |               |         |
|-----------|---------|---------------|---------|
| 1,844,204 | 2/1932  | Clavel .....  | 8/131   |
| 2,184,559 | 12/1939 | Mellor .....  | 8/174   |
| 1,738,946 | 12/1929 | Chapin.....   | 8/149.3 |
| 2,999,002 | 9/1961  | Dayvault..... | 8/94    |

FOREIGN PATENTS OR APPLICATIONS

535,379 4/1941 Great Britain ..... 8/130.1

823,022 11/1959 Great Britain ..... 68/22 A

## OTHER PUBLICATIONS

Hunter, Amer. Dyestuff Reporter, April 12, 1954, pages 236-238.

White, Amer. Dyestuff Reporter, July 31, 1967, pages 591-597.

Primary Examiner—Donald Levy  
Attorney, Agent, or Firm—Glwynn R. Baker

[57] ABSTRACT

An improved process for dyeing textile fabrics from halogenated hydrocarbon solvents which comprises the steps of dyeing, fixing the dyestuff, scouring the dyed textile, removing scour liquor and subsequently subjecting the dyed textile to an atmosphere of steam, preferably superheated steam, under conditions to prevent condensation of any moisture onto or into the emerging textile, thereby to increase the light fastness and wash fastness of the dyed fabric.

3 Claims, No Drawings

**INCREASING DYE FASTNESS OF SOLVENT DYED  
SOLVENT SCOURED DRIED FABRIC BY  
STEAMING**

**BACKGROUND OF INVENTION**

Recently a process has been publicized for solvent dyeing textile materials, woven or unwoven. The process permits rapid dyeing because much less heat is required to remove the dye formulation carrier than when water is employed. However, it has been noticed that some thusly dyed materials are off-color or change hue when exposed to light and/or are washed with detergent. It has been advanced that even though the temperature achieved is high enough and the textile is exposed long enough to such temperatures to fix the dyestuff a phenomenon occurs which affects the "degree of aggregation" of dyestuff, which relates to the physical state of the dye molecule in the fiber.

**BRIEF DESCRIPTION OF INVENTION**

It has now been found that solvent dyed textile material can be stabilized to color change on exposure to light and/or to washing by subjecting the dry, scoured, fixed dyed textile material to steam for from 1 to 10 minutes. Preferably the dyed textile material is brought hot (200° to 250°F.) directly from the solvent recovery zone into a steam zone which is maintained at from about 210°F. to about 240°F. (preferably 215° to 220°F.), and passed through the zone at a rate to prevent the fabric emerging from the zone being wet with any condensate steam.

**DETAILED DESCRIPTION OF INVENTION**

In accordance with the present invention, a solvent-dye formulation was prepared by mixing, e.g., 1 gram of Nabor Orange G Base (C.I. Basic Orange 21, C.I. 48035) in 50 ml. of ethylene glycol monoethyl ether dissolved in 450 ml. of methylene chloride. The so-prepared dye formulation was padded onto a synthetic fabric woven from a yarn containing 70 percent of a copolymer of vinyl chloride and acrylonitrile, 20 percent of a polyacrylonitrile and 10 percent nylon. The dye wetted fabric was passed into and through the vapors of perchloroethylene at a rate to insure the fibers were exposed to the vapors for 30 seconds to assure fixation of the dyestuff. The vapors were at a temperature of 120°C. (248°F.). Any unfixed dye and the unvaporizable glycol ether were removed by subjecting part of the dyed fabric to scouring in cold perchloroethylene and the remainder to scouring in a 0.2 percent aqueous de-

tergent bath and dried.

The solvent scoured fabric was dried in an atmosphere of superheated vapors of perchloroethylene for three minutes. The aqueous scoured fabric took 30 minutes to dry on a heated surface at the 158°F. (70°C)

The solvent scoured textile fabric had a decided reddish shade and was less light fast compared to the aqueous detergent scoured fabric. A portion of the solvent scoured fabric was then subjected to a three-minute treatment in superheated steam at 120°C. (248°F.). The shade of the so-steamed fabric was identical to that of the aqueous detergent scoured fabric and its light fastness was equal.

It is thus seen that the solvent dyeing process can employ a solvent scour and a dry steaming to accomplish the same result obtained by aqueous scouring insofar as light fastness and wash fastness (no change in shade when exposed to water or moisture) are concerned in a much shorter period of time than could be accomplished by use of the heretofore advanced and widely used aqueous scour.

We claim:

1. In a method for improving the light fastness and wash fastness of solvent dyed textiles wherein the dyestuff is applied from a solution or dispersion of the dyestuff in a halogenated hydrocarbon solvent to the textile, the resulting wet textile is subjected to the effect of superheated vapors of a halogenated hydrocarbon solvent maintained at a temperature to fix the dyestuff onto and into the textile, the so-dyed textile which may be still wet with dye formulation solvent or which may be freed thereof is scoured in a halogenated hydrocarbon solvent and thereafter freed of said scour solvent by subjecting the textile to the effect of superheated vapors of the halogenated hydrocarbon solvent, the improvement which consists of subjecting the dry dyed textile after removal of scour solvent to steam at a temperature of from about 110°C. (230°F.) to about 120°C. (248°F.) for from about 1 to 10 minutes under such conditions that no steam condenses on the fabric.

2. The method of claim 1 wherein the steam is at a temperature of from about 110° to about 120°C. and the textile is exposed to the steam for from 1 to 3 minutes.

3. The method of claim 2 wherein the steam is superheated steam.

\* \* \* \* \*